

May 13, 1952

M. A. CHAVANNES ET AL

2,596,128

METHOD AND APPARATUS FOR PRODUCING FINE FIBERS

Filed Oct. 17, 1949

6 Sheets-Sheet 1

Fig. 1



Initial Heating Temperature, °C. Inventors:

Marc A. Chavannes

John C. Elliott

By Zabel & Gutzbaugh

Attorneys

May 13, 1952

M. A. CHAVANNES ET AL

2,596,128

METHOD AND APPARATUS FOR PRODUCING FINE FIBERS

Filed Oct. 17, 1949

6 Sheets-Sheet 2

Fig. 2.



Temperature of Drawing Zone, °C. Inventors:

Marc A. Chavannes

By: John C. Elliott  
Zabel & Britzbaugh  
Attorneys

May 13, 1952

M. A. CHAVANNES ET AL

2,596,128

METHOD AND APPARATUS FOR PRODUCING FINE FIBERS

Filed Oct. 17, 1949

6 Sheets-Sheet 3

Fig. 3.



Hot Bath Temperature  
(Cold Bath Constant at 68°C.)

Inventors:

Marc A. Chavannes

John C. Elliott

By: Zabel & Gutlaugh  
Attorneys

May 13, 1952

M. A. CHAVANNES ET AL

2,596,128

METHOD AND APPARATUS FOR PRODUCING FINE FIBERS

Filed Oct. 17, 1949

6 Sheets-Sheet 4

Fig. 4.



Temperature of Cold Bath  
(Hot Bath Constant at 168-69°C)

Inventors:  
Marc A. Chavannes  
John C. Elliott

By: Zabel & Gutlaugh  
Attorneys:

May 13, 1952

M. A. CHAVANNES ET AL

2,596,128

METHOD AND APPARATUS FOR PRODUCING FINE FIBERS

Filed Oct. 17, 1949

6 Sheets-Sheet 5

Fig. 5.



Inventors:  
Marc A. Chavannes  
John C. Elliott  
By: Zabel & Gitzbaugh  
Attorneys

May 13, 1952

M. A. CHAVANNES ET AL

2,596,128

METHOD AND APPARATUS FOR PRODUCING FINE FIBERS

Filed Oct. 17, 1949

6 Sheets-Sheet 6

Fig. 6



Inventors:  
Marc A. Chavannes  
John C. Elliott  
By: Zabel & Gutlaugh  
Attorneys

## UNITED STATES PATENT OFFICE

2,596,128

METHOD AND APPARATUS FOR PRODUCING  
FINE FIBERS

Marc A. Chavannes, New York, N. Y., and John C. Elliott, Madison, Wis., assignors, by mesne assignments, to Chavannes Synthetic Fibres, Inc., a corporation of Delaware

Application October 17, 1949, Serial No. 121,855

13 Claims. (Cl. 18—1)

1

This invention relates to a method for treating fibers, and more particularly to a method and apparatus for preparing extremely fine fibers from thermoplastic resinous polymers.

Heretofore many synthetic polymers, such as for example, polyvinylchloride, polyvinylidenechloride and copolymers of vinylidenechloride and vinylchlorides, have proved extremely useful in the textile field in the form of oriented fibers. However, a drawback for these fibers has been the difficulty of extruding them in thicknesses of less than about .004 inch.

An object of the present invention is to provide a method for preparing films and fibers of polyvinylidene, or polyvinylchloride or their copolymers, in any desired degree of fineness.

Another object is to produce, as an article of manufacture, exceedingly fine strands of polymers which it has not previously been possible to prepare in such very fine form.

A still further object of this invention is to provide a new method of handling and drawing fibers. Further objects will become apparent as the following detailed description proceeds, reference being made to the accompanying drawings wherein:

Figures 1 through 4 are diagrammatic curves showing the results obtained with a sample of a representative fiber of 10 mil diameter composed of an oriented copolymer of vinylchloride and vinylidenechloride. Figures 5 and 6 are diagrammatic views of two devices for carrying out the process of our invention.

In accordance with our invention in its broad aspect, we first disorient an oriented fiber by heating the fiber to a temperature within the temperature range at which the fiber undergoes plastic flow, and then either at the plastic flow temperature or below this temperature draw the fiber to a substantial extent, as for example, 100% of its length or greater, and then repeat the procedure of disorienting and drawing.

In accordance with a preferred embodiment of our invention, the fiber, after being heated and allowed to shrink, is first drawn in the plastic flow temperature range to a small extent, as for example, to its length before shrinkage, or from 50% to 200% of its length after shrinkage, then supercooled below the plastic flow range and drawn to a larger extent, as for example, 400% to 5000% of its original length at the lower temperature. The entire sequence of operations may then be repeated for the best results.

We may start with fibers of 10-12 mils diameter, bring such fibers to 2 mil diameter in one

series of operations, and then to  $\frac{1}{2}$  mil diameter in the second set of operations. Fibers made of copolymer of vinylidenechloride and vinylchloride may readily be converted by our process to fibers of 1 mil diameter and lower. Thus by a sequence of disarrangement and drawing operations, it is possible to draw a heavy extruded textile fiber to almost any desired degree of fineness.

In accordance with another embodiment of our invention we heat a fiber comprising a copolymer of vinylchloride and vinylidenechloride for several seconds at 150° to 205° C. to produce disarrangement of the micellar structure, allowing it to shrink freely. We then draw it at the same temperature range, or at a lower temperature if desired, to approximately its original length. While holding it at this length, we then submit it to a temperature of 38° to 80° C. and then draw it to 10 to 50 times its original length at this temperature, producing a corresponding reduction in the thickness of the fiber. This fiber of reduced thickness may then be subjected to a repetition of the same process and drawn again to 10 to 50 times its length, i. e., 100 to 2500 times its original length. Thus it is possible by further repetition of this process to draw the fibers ad infinitum to any desired degree of fineness, in a continuous process.

For further explanation of the process, we refer to Figure 5, which is a diagrammatic view of a device embodying the principles of our invention. In Figure 5, fiber 1 enters the device at triple-rolls (hereinafter, "rolls") 2 from which it passes into oven 3, cut away to show electric heating wire 4, insulation 5 and rolls 6. Rolls 2 maintain any tension in the fiber which may be necessary prior to its entry into the device. The fiber passes from rolls 2 to rolls 6 which turn at a slower rate and allow fiber 1 to have substantially no tension and to shrink freely between rolls 2 and 6. The fiber then passes to rolls 7 which turn faster than rolls 6, drawing the fiber to approximately the length it had prior to entering the machine. Fiber 1 then enters oven 8 maintained at a lower temperature than oven 3 by electric resistance wire 9. The fiber passes then through rolls 10 which turn at a faster rate, drawing the fiber to 4 to 50 times its original length. Fiber 1 then passes over idler roll 11 and may then pass on to other processing machinery or to storage or may be subjected to repetition of the process just described, as for example, in the device shown, where the fiber passes over idler roll 12 to rolls 13 which turn at sub-

## 3

stantially the same rate as rolls 10. The fiber then enters oven 14 maintained at substantially the same temperature as oven 3. Oven 14 is cut away to show electric resistance wire 15, insulation 16 and rolls 17. In this oven it passes through rolls 17 which turn at a slower rate to allow the fiber to shrink freely between rolls 13 and 17. The fiber then passes to rolls 18 which turn faster than rolls 17 and draw the fiber out to approximately its original length. From rolls 18 fiber 1 then passes to oven 19 maintained at substantially the same temperature as oven 3. The fiber then passes through rolls 20 which turn at a faster rate than rolls 18, drawing the fiber to 4 to 50 times the length it had upon entering oven 14. The fiber then passes over idler rolls 21, 22 and 23 and may then pass on to other operations or may be subjected to further repetitions of the process of this invention, as described.

Another form of device for carrying out our process is shown in Fig. 6 wherein the reference numerals 25 and 26 designate a supply spool and a wind up spool, respectively, for a fiber 21. The fiber in passing from the supply spool to the wind up spool passes through a plurality of pairs of rubber covered rollers 28, 29, 30 and 31. These rollers are driven at various peripheral speeds by means of worms 32, 33, 34 and 35, respectively, the worms being mounted on a common worm shaft 36. Suitable gearing 37, 38, 39 and 40, respectively, is interposed between the pairs of rollers and their respective worms. Between rollers 28 and 29 there is disposed a heating chamber 41 and a cooling chamber 43. The heat may be developed by any suitable means, such as a resistance wire or by superheaters using radiant heat, or the fiber may be heated by a blast of hot air which is supplied to the chamber 41 by means of a pipe 42, as shown. Similarly, the fiber may be cooled by supplying coil air to the chamber 43 through pipe 44. A similar heating chamber 45 and cooling chamber 47 are provided between rollers 29 and 30, the chambers being provided with supply pipes 46 and 48, respectively. A third set of heating and cooling chambers 49 and 51 are provided between rollers 30 and 31, together with the supply pipes 50 and 52, respectively.

In operation, the rollers 28 may be driven by means of worms 32 and gears 37, at 100 revolutions per minute so that the fiber is fed into and through the chambers 41 and 43. In the chamber 41 the fiber is heated to approximately 170° C. which causes shrinkage, after which the fiber is cooled as it passes through cooling chamber 43, so that at the time the fiber is engaged by the rollers 29, it is chilled. As above indicated, the cooling may be effected by supplying cold air of a temperature of approximately 10° C. through the supply pipe 44. The rollers 29 are driven at substantially 50 revolutions per minute in order to allow for the shrinkage which occurs in the heating chamber 41. The rollers 30 may be driven at 100 revolutions per minute so that in passing through the heating and cooling chambers 45 and 47, respectively, the fiber is restored to its original length. In the heating chamber 45 the fiber is heated to approximately 170° C. and it is suitably cooled in chamber 47 by cold air, at approximately 10° C., which is supplied thereto.

The main drawing operation occurs as the fiber is drawn through heating chamber 49 and cooling chamber 51, and the last pair of rollers 31 may be driven at the speed necessary to effect

the desired amount of drawing. For instance, the latter rollers may be driven at 600 revolutions per minute; the fiber may be heated in chamber 40 up to 60° C.; and, it may then be cooled in cooling chamber 51 by cold air supplied thereto at a temperature of approximately 10° C.

The above described device is illustrative only since it will be appreciated that the speeds and temperatures are subject to considerable variation depending on the particular results to be obtained. In the above illustration, it is assumed that the diameter of the rollers is somewhat less than 4 inches so that the circumference of the rollers is substantially 1 foot. Thus, rollers 28 rotating at 100 revolutions per minute serve to feed the fiber at 100 feet per minute.

Suitable means may be provided for driving the supply and wind up spools 25 and 28 at the proper rates of speed.

In each stage of the process it will be observed that the filament is chilled by cold air so that it is never touched by the rollers when it is in its heated condition.

Results obtained with fibers of a copolymer of vinylidenechloride and vinylchloride (Saran) are shown by reference to Figures 1, 2, 3 and 4.

Fig. 1 is a graph wherein the initial heating temperature of the fiber in a hot bath is plotted against the maximum length to which the fiber could be drawn.

Fig. 2 is a graph wherein the temperature of the drawing zone in which the fibers are drawn is plotted against the maximum length to which the fiber could be drawn.

Fig. 3 is a graph wherein the hot bath temperatures of from 155° C. to 206° C. for the fibers are plotted against the maximum inches of stretch of the fiber. After disorienting the fiber in the hot bath and stretching to 4 inches, the fiber was drawn to 21 inches in a cold bath maintained at 68° C., removed and the drawing continued in air until the fiber broke.

Fig. 4 is a graph showing the effect of varying the cold bath temperature from 40° C. to 80° C., the hot bath being maintained at 168-169° C. The disorienting and stretching procedure was the same as described for Fig. 3.

It is not essential to the invention how the heating is arranged. We may employ induction heating methods, hot air, radiant heat, or we may immerse the fibers and pass them through baths of heated oil or any other heat transfer medium which does not attack or interfere with the fibers.

In this manner, the fibers are drawn to any desired degree of fineness.

The applicability of the invention will become further apparent from the following specific examples which are given here by way of illustration only, and not in any sense whatever by way of limitation. The parts shown in the examples are by weight.

## Example I

A two inch length of pigmented fiber composed of a copolymer containing 85 percent polyvinylidenechloride and 15 percent polyvinylchloride and having a thickness of .012 inch was immersed for 2 seconds in a bath of oil maintained at 173° C. while being allowed to shrink freely.

While still in the same bath it was then drawn to its original length and was then immediately transferred to an oil bath maintained at 68° C. and drawn, in the bath, at the rate of 6 feet per minute to a length of 70 inches. The resulting fiber had a diameter of .002 inch.

## 5

## Example II

A two inch length of pigmented fiber composed of a copolymer containing 85 percent polyvinylidenechloride and 15 percent polyvinylchloride and having a thickness of .012 inch was immersed for 2 seconds in a bath of oil maintained at 155° C. while being allowed to shrink freely. While still in the same bath it was then drawn to its original length and was then immediately transferred to an oil bath maintained at 74° C. and drawn, in the bath, at the rate of 6 feet per minute to a length of 21 inches. The resulting fiber had a diameter of .0015 inch.

## Example III

A two inch length of pigmented fiber composed of a copolymer containing 85 percent polyvinylidenechloride and 15 percent polyvinylchloride and having a thickness of .012 inch was immersed for 2 seconds in a bath of oil maintained at 203° C. while being allowed to shrink freely. While still in the same bath it was then drawn to its original length and was then immediately transferred to an oil bath maintained at 68° C. and drawn, in the bath, at the rate of 6 feet per minute to a length of 39 inches. The resulting fiber had a diameter of .0015 inch.

## Example IV

A two inch length of pigmented fiber composed of a copolymer containing 85 percent polyvinylidenechloride and 15 percent polyvinylchloride and having a thickness of .012 inch was immersed for 2 seconds in a bath of oil maintained at 190° C. while being allowed to shrink freely. While still in the same bath it was then drawn to its original length and was then immediately transferred to an oil bath maintained at 40° C. and drawn, in the bath, at the rate of 6 feet per minute to a length of 20 inches. The resulting fiber had a diameter of .0018 inch.

## Example V

A 1000 foot length of a pigmented fiber composed of a copolymer containing 85 percent polyvinylidenechloride and 15 percent polyvinylchloride and having a thickness of .012 inch was wound on a spool. The spool was then mounted in such a manner that the fiber could be drawn from it and passed through a device comprising two oil baths and five sets of rollers which gripped the fiber strongly and three idler rolls, substantially as shown in Figure 1. The first bath was maintained at 172° C. and the second at 79° C. with electric heaters and controlling thermostats. The rolls were driven by a series of V-belts and chains and sprockets from a variable speed drive driven by an electric motor. The fiber was passed through the apparatus at a rate which permitted it to shrink freely in the high temperature bath for 2.2 seconds and to be drawn to 0.96 times its original length, in the high temperature bath, in 1 second. The fiber then passed from the hot bath into the cold bath and was drawn therein to 10.6 times its original length. The resulting fiber had a diameter of .002 inch.

## Example VI

A two inch length of fiber composed of a copolymer containing 90 percent polyvinylidenechloride and 10 percent polyvinylchloride and having a thickness of .015 inch was immersed for 3 seconds in a bath of oil maintained at 225° C. while being allowed to shrink freely. While still

## 6

in the same bath it was then drawn to approximately its original length and was then immediately transferred to an oil bath maintained at 100° C. and drawn, in the bath, at the rate of 3 feet per minute to a length of 56 inches. The resulting fiber had a diameter of .002 inch.

## Example VII

A two inch length of a pigmented polyethylene fiber having a thickness of .012 inch, of the type sold commercially as "Avisco Type B" was immersed for 15 seconds in a bath of oil maintained at 132° C. while being allowed to shrink freely. While still in the same bath it was then drawn to slightly over  $\frac{1}{2}$  its original length and was then immediately transferred to a bath maintained at 100° C. and drawn to 7.0 inches in length. It was then re-immersed in the 132° C. bath for 5 seconds while being allowed to shrink freely and was then transferred to the 100° C. bath and drawn to 8.5 inches. The resulting fiber had a diameter of .0041 inch.

The above examples by no means exhaust the different possible applications of our invention. They have been shown by way of illustration only and not in any sense by way of limitation.

The examples have shown the use of polyethylene and of copolymers of vinylchloride and vinylidenechloride as the synthetic resins comprising fibers to which our invention is applicable. These are not to be considered limiting in any respect; the invention is not confined to these particular resins. Fibers formed from polyvinylchloride, polyvinylidenechloride and resinous copolymers formed by the copolymerization with vinylchloride or vinylidenechloride or copolymers of vinylchloride and vinylidenechloride of such other monomers as may be so copolymerized are also the subject of this invention. Such copolymers include for example; copolymers of vinylacetate or vinylbutyral with vinylchloride, vinylidenechloride or vinylchloride and vinylidenechloride, copolymers of acrylic acid esters or methacrylic acid esters with vinylchloride, vinylidenechloride, or vinylchloride and vinylidenechloride, and copolymers of styrene or dichlorostyrene with vinylchloride, vinylidenechloride, or vinylchloride and vinylidenechloride. The bromides or other halide compounds corresponding to the above chloride compounds may also be used.

The examples have shown the use of several methods for carrying out the heat treatment of a fiber according to our invention, but these are not to be considered limiting in any way. Our invention contemplates the use of any method of heating which can be applied to a synthetic resin fiber and the application of heat to fibers in both continuous and non-continuous devices. Such heating may be accomplished in the following ways, for example: with an oven, with a liquid bath, with induction coils, with radiant bulbs or surfaces, or by passing the fiber over heated rollers.

We prefer to carry out the initial heating step in the process of our invention at temperatures of 130° to 240° C. for a duration of 2 to 15 seconds. Useful results, however, are obtained at temperatures of 120° to 245° C. and durations of .5 to 30 seconds. We prefer to draw the fibers to at least  $\frac{1}{2}$  their original length and to not more than 1 $\frac{1}{2}$  times their original length while still at the temperature of the initial heating, but useful results are obtained if the fibers are drawn to  $\frac{1}{4}$  to 2 times their original length at this

temperature. We prefer to maintain the temperature of the second or low-temperature zone, in which the fibers are drawn to 4 to 50 times their original length, at 35° to 110° C. but useful results are obtained at 30° to 220° C. Satisfactory results are obtained if the drawing steps are carried out at drawing rates of 1 to 50 feet per minute but best results are obtained if the drawings are carried out in the preferable range of 3 to 25 feet per minute. The rates shown by the examples are not limiting.

Figures 1 and 2 show, diagrammatically, the result of applying this invention to .012" diameter fibers composed of a copolymer containing 85 percent polyvinylidenechloride and 15 percent polyvinylchloride. The method of this invention was applied to samples of such fibers and various temperatures were used for the different steps of the process.

The curve of Figure 1 shows the length to which such fibers could be drawn at 6 feet per minute at 68° C. after being immersed for a period of 2 seconds in a bath of oil held at various temperatures while being allowed to shrink freely and after then being drawn to approximately their original length at the same temperature. Two sharp peaks are observed in this curve; these occur at 173° C. and 190° C. and fibers could be drawn to 3360 and 3220 percent of their original length, respectively, after initial heating and drawing at these temperatures.

The curve of Figure 2 shows the length to which such fibers could be drawn at various temperatures, using a drawing rate of 6 feet per minute, after being immersed for 2 seconds in an oil bath held at 168° to 169° C. while being allowed to shrink freely and then being drawn to approximately their original length at the same temperature. This curve also has two sharp peaks. These are at 68° C. and 74° C.; fibers could be drawn to 3450 and 3500 percent of their original length, respectively, at these temperatures.

While we do not wish to commit ourselves to any particular theory as to the mode of function of our invention, it is our belief that the initial heating of the oriented fiber, which is accompanied by extreme shrinking of the fiber, produces disorientation of the polymeric molecules, effecting disarrangement of the molecular configuration and micellar arrangement. Drawing the fiber to 1/2 to 1 1/2 times its original length at close to this same temperature is thought to cause some chemical unbonding of bonds which are weakened by the heating. Subsequent drawing to very great lengths at lower temperature to produce a very thin fiber of reoriented molecules is made possible by this disorientation and unbonding.

Optimum temperature conditions for carrying out the initial heating and slight drawing occur above the softening point of the resin. Optimum temperatures for the subsequent drawing to great length are found below the softening point.

It is to be fully understood that the invention is broad in scope, and is to be restricted only by the claims, in which it is our intention to cover all novelty inherent in the invention as broadly as possible, in view of prior art.

Having thus disclosed our invention, we claim:

1. The process of producing a fine fiber from a thicker fiber of an oriented thermoplastic

resinous polymer which comprises disorienting the fiber by heating the fiber to a temperature at which the fiber undergoes plastic flow, allowing the fiber to shrink, drawing the fiber at a temperature within the plastic flow temperature range after the fiber has undergone shrinkage, cooling the fiber to below the minimum temperature of plastic flow, and drawing the fiber at said lower temperature to a greater extent than at said higher temperature.

2. The process for producing a fine fiber composed of a copolymer of vinylidenechloride and vinylchloride which comprises heating an oriented fiber of said copolymer at 150° C. to 205° C. for 2 to 15 seconds with the fiber being allowed to shrink freely; drawing said fiber to 1/2 to 1 1/2 times its original length at approximately the same temperature; and then drawing said fiber at 38° C. to 80° C., increasing its length 3 feet per minute at 25 feet per minute, to 10 to 50 times its original length.

3. The process for producing a fine fiber comprising a copolymer of vinylchloride and vinylidenechloride which comprises heating an oriented fiber comprising a copolymer of vinylchloride and vinylidenechloride at 120° C. to 245° C. for 0.5 to 30 seconds with said fiber being allowed to shrink freely; drawing said fiber to 1/4 to 2 times its original length at approximately the same temperature; and then drawing said fiber at 30° C. to 220° C., increasing its length 1 foot per minute to 50 feet per minute, to 4 to 50 times its original length.

4. Apparatus for the processing of fibers or the like comprising a plurality of successive means for engaging and feeding a continuous filament, thereby providing a path for the advance of said fiber, means disposed along said path between the first two of said feeding means for heating said fiber to cause shrinkage thereof, driving means for operating the second one of said feeding means at a slower speed than the speed at which said first feeding means is driven to compensate for said shrinkage, driving means for operating a third one of said feeding means at substantially the same speed as that at which said first feeding means is driven in order to draw said fiber to approximately its original length, driving means for operating a fourth one of said feeding means at a substantially greater speed than that at which said first feeding means is driven in order to draw said fiber to a substantially greater extent than that at which it is drawn by said third one of said feeding means, means disposed along said path between said third and said fourth feeding means for maintaining said fiber at a temperature substantially less than the temperature to which it has been raised by said first mentioned heating means, and heating means disposed along said path between said second and third feeding means in order to heat said fiber during the first of said drawing operations.

5. Apparatus as claimed in claim 4 provided with cooling means between each of said heating means and the succeeding feeding means whereby said fiber is chilled prior to the time that it is engaged by said feeding means.

6. Apparatus for producing a fine fiber comprising four sets of fiber feeding rollers, three separate fiber heating means, one of said heating means being disposed between each adjacent pair of sets of rollers, means for driving said first and third sets of rollers at approximately the same peripheral speed, means for driving said second

set of rollers at a peripheral speed less than that at which said first and third sets of rollers are driven, and means for driving said fourth set of rollers at a speed greater than the speed at which said first and third sets of rollers are driven.

7. Apparatus as claimed in claim 6 in combination with three separate fiber chilling means, one fiber chilling means being disposed in front of each of said second, third and fourth sets of rollers whereby a continuous fiber passing through each of said successive heating means will be chilled prior to the time that it is engaged by successive sets of rollers.

8. Apparatus as claimed in claim 6 in combination with common driving means for all of said sets of rollers.

9. The process of claim 1 wherein the polymer is polyvinylchloride.

10. The process of claim 1 wherein the polymer is a copolymer containing polyvinylchloride.

11. The process of claim 1 wherein the polymer is a copolymer of vinylchloride and vinylidenechloride.

12. The process of claim 1 wherein the polymer

## 10

is a copolymer of vinylchloride and vinyl acetate.

13. The process of claim 1 wherein the polymer is polyethylene.

MARC A. CHAVANNES.  
JOHN C. ELLIOTT.

## REFERENCES CITED

The following references are of record in the file of this patent:

## UNITED STATES PATENTS

| Number    | Name               | Date          |
|-----------|--------------------|---------------|
| 2,161,766 | Rugeley et al.     | June 6, 1939  |
| 2,183,602 | Wiley              | Dec. 19, 1939 |
| 2,239,780 | Fikentscher et al. | Apr. 29, 1941 |
| 2,354,744 | Dreyfus            | Aug. 1, 1944  |
| 2,367,173 | Martin             | Jan. 9, 1945  |
| 2,476,830 | Spencer            | July 19, 1949 |

## OTHER REFERENCES

Sherman and Sherman: "The New Fibers," Van Nostrand, New York, 1946, page 98. (Copy in Division 15.)